

## UNITED STATES PATENT OFFICE

EDNA A. HASTINGS, OF CLEVELAND, OHIO, ASSIGNOR TO HARRY E. SCHREIBER, OF CLEVELAND, OHIO

## LAMP SHADE AND METHOD OF MAKING THE SAME

No Drawing.

Application filed July 18, 1930. Serial No. 468,998.

This invention relates to a method of treating paper for producing variegated and ornamental color effects thereon, whereby it may be adapted for use as a lamp shade. Lamp shades of this character are commonly known as parchment shades, and so far as I am aware, have heretofore been made by soaking a relatively expensive paper in water until it is soft and pliable. It is then dried, treated 10 with mineral oil, and then creased or crumpled to obtain a crackled effect. Thereafter, the decoration is applied, and the paper is assembled on the frame. A finish coating of shellac is then applied on the outer surface of 15 the shade.

I have found however, that this method of making a lamp shade is objectionable, for unsightly white spots appear on the shade, after it has been standing for about a month, 20 and that such spots cannot be removed by subsequent treatment. Accordingly, the shades are rendered unsalable. It is my belief that the objectionable discoloration is due principally to the character of the oil which 25 has been used, and also to the fact that the paper may hold occluded moisture, which has not been entirely removed before the oil has been applied. It is also my belief that the alcohol in the shellac attacks the mineral 30 oil, and thereby tends to produce objectionable discoloration, although discoloration has occurred even though the shellac has not been used. It is desirable however to apply a finish coating of shellac in order to enhance the 35 finished appearance of the shade.

An object of my invention therefore, is to provide a method of treating paper, which will not only eliminate the objectionable discoloration, but which will also permit the 40 shade to be made from relatively inexpensive paper, and in a materially reduced period of time.

I carry out my invention by cutting the pattern from a grade of paper, which is commercially known as manila 2-X and which is a relatively cheap grade of craft paper. Heat is applied, as by an ironing operation, to drive off occluded moisture, and then the oil is applied to each side of the paper. I 45 have found that best results can be obtained

by utilizing castor oil, and that the oil has greater penetrating properties if it is mixed with denatured alcohol. For this purpose, I have found that the ingredients can be mixed in the proportions of substantially two-thirds castor oil, and one-third denatured alcohol. If desired however, the castor oil can be used without the solvent, but when so used, it is difficult to handle as it will not flow readily.

After the paper has been so treated, it is suspended until the alcohol is evaporated. If additional translucency is desired, heat is applied on one side with a very hot iron, and then the surface is brushed immediately with clear castor oil while the paper is still hot. The heat may, if desired, be applied after instead of before the second application of oil to produce substantially the same results. Surplus oil is then removed by placing the 50 paper between layers of absorbent paper. If a crackled effect is desired on the shade, the paper is then bent along the desired lines, and in such manner that the concave side of the creases are disposed on the outer side.

The creases may then be smoothed out with a medium hot iron and additional clear castor oil may be applied to those regions where additional translucency is necessary. A decoration can now be applied to the surface 55 either by tinting or by painting a figure or character thereon. Then the paper can be fastened onto the frame in the usual way, and a coating of shellac applied to protect the decoration.

I have found that shades made in accordance with my method are entirely free from the presence of objectionable spots, even though they are made with or without the application of shellac as a finish coating. Furthermore, I have found that these shades can be stored indefinitely, and that they can be made from a relatively cheap grade of manila paper. Furthermore, by eliminating the water treatment, I have materially reduced 60 the time in which the shades can be made.

I claim:

1. A method of treating paper for making a lamp shade, comprising cutting a paper pattern, applying heat to evaporate occluded

moisture, applying a coating of vegetable oil mixed with a solvent, evaporating the solvent, applying intense heat, and then applying a coating of vegetable oil to obtain additional 5 translucency.

2. A method of treating paper for making lamp shades, comprising cutting a paper pattern, applying a mixture of castor oil and alcohol thereto, allowing the alcohol to evap-

10 orate, applying heat, applying a coating of vegetable oil while the paper is hot, creasing the paper, and then applying a decoration thereto.

3. A method of treating paper for making 15 a lamp shade, comprising cutting a paper pattern, ironing it, applying a mixture of castor oil and alcohol to each side of the paper, suspending the paper until the alcohol is evaporated, applying intense heat to one

20 side of the paper, applying a coating of castor oil, while the paper is hot, removing surplus oil, creasing the paper, and then applying a decoration thereto.

4. A method of treating paper for making 25 lamp shades comprising cutting a paper pattern, applying a mixture of castor oil and a solvent thereto, allowing the solvent to evaporate, applying a second layer of castor oil and subjecting the second layer to intense

30 heat until it is impregnated into the paper.

In testimony whereof I hereunto affix my signature.

EDNA A. HASTINGS.

35

40

45

50

55

60

65